# EUROPEAN PATENT APPLICATION

(11) **EP 0 267 299 A1**
(43) Date of publication of application: **18.05.1988**
(21) Application number: 87903412.2
(22) Date of filing: 19.05.1987
(51) Int. Cl.: G03C 7/00, G03C 7/02, G03C 7/16, G03C 1/86

(54) **HIGH-QUALITY POSITIVE SILVER HALIDE COLOR PHOTOGRAPHIC MATERIAL**

(30) Priority: 20.05.1986 JP 11583986
(71) Applicant: KONICA CORPORATION, Tokyo 163 (JP)
(72) Inventor: KOMATSU, Hajime, 28, Horinouchi Odawara-shi Kanagawa 250 (JP); INAHATA, Hideki, 28, Horinouchi Odawara-shi Kanagawa 250 (JP)
(74) Representative: Gille Hrabal Struck Neidlein Prop Roos
(86) International application number: PCT/JP1987/000318
(87) International publication number: WO 1987/007399

(57) **Abstract**

A positive silver halide color photographic material which comprises an 80-µm to 150-µm thick reflective support having provided thereon a red-sensitive negative silver halide emulsion layer, a green-sensitive negative silver halide emulsion layer, and a blue-sensitive negative silver halide emulsion layer capable of forming cyan, magenta, and yellow images, respectively, with a dye image density given as a negative function of image exposure quantity. When the support has unevennesses of 1mm to 15 mm in diameter on the emulsion layer side, the depth of the unevennesses are not more than 4 µm. This photographic material provides a thin, high-quality positive image.

## Description

### FILED OF THE INVENTION

The present invention relates to a positive-type silver halide color photographic light-sensitive material forming a dye image by converting an amount of image exposure into a negative function. In particular, according to the invention, the similar light-sensitive material can be used as a high-quality, positive-type light-sensitive material suitable for duplicating an original picture containing image information such as characters, pictures and the like.

### BACKGROUND OF THE INVENTION

In duplicating characters, designs and sketches, and in cataloging merchandise, photographic light-sensitive materials are used. For this purpose, a negative-positive process, wherein a negative image is firstly formed on a negative film, then the image is converted into a positive image, is usually carried out. Involving developing two times, such a negative-positive process incurs much labor, and, disadvantageously, more cost, since it requires the cost for preparing a negative.

To solve such an disadvantage, as a means to form a positive image directly, a reversal silver halide color photographic light-sensitive material using reversal developing, as well as a silver dye bleach-type silver halide color photographic light-sensitive material using a catalyst of oxidized silver, are known in the art. In addition, those known in the art include the electrophotography using electrostatic transfer process.

Being extremely simple, and being capable of producing a thin duplicate, the electrophotography is a useful process. However, this process fails to provide a sufficient gradation tone to represent the shade of original image, and, accordingly, it is quite difficult to provide a duplicate with a high definition.

At the same time, a process using a positive silver halide light-sensitive material., wherein a negative silver image is formed by the monotone primary developing using an oridinary silver halide emulsion, then the image is treated to form a positive color image, is a technique suitable for producing a high-quality duplicate. However, with this technique, a thin support (substrate) comparable to one used in the electrophotography has not yet been put into a practical use.
Compared to the negative-positive silver halide silver halide color photographic light-sensitive material, having a shorter processing time in terms of the total processing system, and being capable of providing high quality images, the reversal type and silver dye bleach type silver halide color photographic light-sensitive materials have been used for special application, however, the support used therein is substantially thick.

When filing photographic papers bearing duplicated images, the thickness of support disadvantageously results in a bulky file. Futhermore, when used for a design work, the thickness of photographic paper placed on a paper mount readily forms a shadow, causing much inconvenience.

For these reasons, the introduction of a positive silver halide color photographic light-sensitive material using a thin support is necessary.

In view of this, the inventors have continued the improvement to provide a positive silver halide color photographic light-sensitive material using a thin support, that is. for example, the reversal type or silver dye bleach type silver halide color photographic light-sensitive material.

In the course of the study, the inventors have learned that, with a thin support having a thickness less than 150 µm, the uneveness of coat which did not pose serious disadvantages with a conventional positive type silver halide color photographic material using a thick support occurs, and, subsequently, visually offensive uneveness of image density develops on a print after the developing, and that the similar material having such a thin support cannot be commercially used.

In other words, with a negative silver halide color photographic light-sensitive material with which the density of dye image is determined as a positive function in proportion to the exposure of image, such a visually offensive uneveness in density does not readily occur. In contrast, with a reversal type or silver dye beach type positive silver halide color photographic light sensitive material with which the density of dye image is determined as a negative function in proportion to the exposure of image, such a visually offensive uneveness in density readily occurs.

The inventors have learned that such an uneven density closely relates to both the thickness of support and the type of light-sensitive material formed on the support.

Additionally, with a negative silver halide color photographic light-sensitive. material, which is a color photographic paper onto which an image on a negative film is printed, a yellow dye image whose density is not readily judged with human vision is usually formed in a silver halide emulsion layer nearest to a support whereupon uneveness of coat often occurs. Accordingly, a visually offensive uneven density seldom occurs even if a film of coat is unevenly formed.

### SUMMARY OF THE INVENTION

The present invention has been made to solve the above-mentioned disadvantages, therefore, it is the object of the invention to provide a positive silver halide color photographic light-sensitive material free from a visually offensive uneven density, such as a reversal type or silver dye bleach type positive silver halide color photographic light-sensitive material.

More specifically, the object of the invention is to provide a positive silver halide color photographic light-sensitive material, with which a positive image can be directly formed having a thin support suitable for filing and design work.

The light-sensitive material according to the invention is a positive silver halide color photographic light-sensitive material, with which a dye image density is determined as a negative function proportional to the amount of image exposure, comprising a reflective support, provided thereon, a negative type red-sensitive silver halide emulsion layer to form a cyan dye image, a negative type green-sensitive silver halide emulsion layer to form a magenta dye image, and a negative type blue-sensitive silver halide emulsion layer to form a yellow dye image, whereby the thickness of the reflective support is 80 to 150 µm, and when the surface of support where the silver halide emulsion layers are disposed have irregularities whose diameters range at least one to 15 mm, the depths of irregularities are limited to less than four µm, and, accordingly, this arrangement ensures the attainment of the invention.

### BRIEF DESCRIPTION OF THE DRAWINGS

Fig. 1 is a diagramatic cross section illustrating a support used in the present invention;
Fig. 2 illustrates the irregularities on a support used in one example embodying the invention, and;
Fig. 3 illustrates a copying apparatus using a positive type silver halide color photographic light-sensitive material according to the invention.

### DETAILED DESCRIPTION OF THE INVENTION

According to the invention, the depths of the irregularities are, as mentioned previously, less than four µm, preferably, less than three pm, and, more favorably, less than two µm.

With a support according to the invention, when there are irregularities having the diameters at least one through 15 mm on the support surface where emulsion layers are provided, the depths of the irregularities are limited to less than four µm. According to the invention, the diameters of irregularities are same as the distances between neighboring waves. For example, in Fig. 1, when several waves appear in a repetitive pattern, the distances W₁, W₂ and W₂, between neighboring valleys are called the diameters of irregularities or corresponding waves.

In a close view, the surface of a support in Fig. 2 is a very smooth and has minute irregularities in a continuous pattern. However, when viewed from more distant point, the same surface may have, as shown in the figure, larger waves whose diameters being approximately ten mm. In this case, with the waves having diameters less than one mm being ignored, the waves each more than one mm distant neighboring waves are sampled, as shown in the figure, whereby the distances between neighboring valleys are designated the diameters of irregularities. Accordingly, W₁ and W₂' are called the diameters of the corresponding waves.

The inventors have learned that, if the diameters of irregularities are smaller than one mm or larger than 15 mn, a visually offensive uneven density due to the uneveness of coat film is not readily recognizable even if the depths of the irregularities are larger than four pm. Also, when the diameters of irregularities range from one to 15 mm, especially, two to five mm, and if some of the depths of irregularities exceed four µm, a visually offensive uneven density occurs, even if the sizes of the irregularities are substantially identical, thus often deteriorating the quality of print.

According to the invention, the depth of irregularity means, if the irregularities are ruggedly shaped, the greatest depth. For example, in Fig. 1, the depth of the leftmost irregularity is hτ, while the neighboring rugged-shaped irregularity has two theoretical depths, h₂ and h₃. In this case, however, since h₂ is greater than h₃, the greater depth h₂ is regarded as the depth of this irregularity. Similarly, with the next irregularity, since hs is greater than h₄, its depth is hs. h₆ is the depth of the rightmost irregularity.

This description also applies to Fig. 2.

According to the invention, the depths of the irregularities are less than four µm. As a means to measure such irregularities, a device known as a micro-thickness meter or a surface roughness tester can be used. For this purpose, the measuring head should be of a stylus and the area of contact should be sufficiently small in compliance with the surface roughness.

The aforesaid reflective support according to the invention has excellent smoothness and, accordingly, provides a high quality image.

The reflective support used in the invention can be obtained by using various means. Such means are as follows: to intensify the sifting of pulp, so as to decrease the floes of pulp; to increase the amount of sizing agent; to strongly press and squeeze the surface of already formed pulp sheet with a calender roller; to apply a white pigment such as barium sulfate, zinc oxide, imgnesium oxide and the like onto the surface of pulp sheet; and others. It should he noted that more careful operation is usually necessary to improve the smoothness of thin paper support than preparing a thick paper support with the above-mentioned means. In other words, the precautions such as to use a calender pressure larger than that for a thick paper support, to increase the amount of sizing agent, to increase the amount of coating agent, and the like are necessitated.

Onto the surface of a paper support prepared in this way and accordingly having satisfactory smoothness is applied fused polyolefine by means of the extrusion coating process so as to form a water-resistant film. This provides a polyolefine- laminated paper having satisfactory smoothness.

with still another means a reflective support is prepared, wherein polypropylene into which a small amount of filler having been added is fused, then drawn into a paper-like sheet by extrusion, so as to prepare an opaque support. Additionally, a support may be prepared by bonding together two to five sheets of the above drawn polypropylene with the dry- lamination process so as to control the thickness and opacity of support. If a support is provided with a subbing layer, a support including a subbing layer is called the support of the invention.

now, the negative-type silver halide emulsion used to form the silver halide emulsion layers according to the invention is described below.

A composition of silver halide contained in the emulsion is arbitrarily selected, and various types of silver halide can be used for this purpose. However, the preferred component is silver chloro-bromide, silver bromo-iodide or silver chloro-iodide, or the mixture containing these silver halides.

The preferred particle diameter of silver halide particles contained in the emulsion is 0.3 to 1.5 m. There is no specific limitations on the crystal configuration and crystal habit of the silver halide particles being used. In relation to the crystal habits, those preferably used are the cubic, octahedral, tetradecahedral, twin and tabular crystals.

The preparation process for the emulsion may be any of the acid process, neutral process, alkali process, ammonia process and the like: Also, any of the normal precipitation method, reverse precipitation method and double-jet precipi.ta- tion method can be used. Additionally, the pAg controlled double jet precipitation method or the conversion method for a multi layer-structured type emulsion may be used.

In providing the photographic light-sensitive material of the invention, a higher sensitivity emulsion layer and a lower sensitivity emulsion layer may be disposed correspondingly as the upper layer and the lower layer, or these emulsions are blended together to form one layer.

The positive-type silver halide color photographic light-sensitive material of the invention comprises areflective support, provided thereon, a negative-type red-sensitive silver halide emulsion layer to form a cyan dye image, a negative-type green-sensitive silver halide emulsion layer to form a magenta dye image, and a negative-type blue-sensitive silver halide emulsion layer to form a yellow dye image.

The useful yeellow dye forming couplers include benzoy- lacetanilide type and pyvoloylace tanilide type couplers, as well as the bivalent yellow coupler in which a so-called split-off group being capable of splitting off by the coupling reaction is, as a substituent, bonded to a carbon atom in the coupling position.

The useful magenta dye forming couplers include 5-pyrazolone, pyrazolotriazole, pyrazolynobenzimidazole and indazolone magenta couplers, as well as the bivalent magenta coupler having a split-off group.

The useful cyan dye forming couplers include phenol, naphthol and pyrazoquinazolone cyan couplers, as well as the bivalent cyan coupler having a split-off group.

Any of these couplers may be arbitrarily used, and there is no specific limitation on the method of use, the amount of addition, and others.

One example of positive-type silver halide color photographic light-sensigive material of the invention comprises a support, sequentially disposed on the one side thereof by means of coating, a red-sensitive negative-type silver halide emulsion layer containing cyan coupler, a green-sensitive negative-type silver halide emulsion layer containing magenta coupler, a yellow filter layer, and a blue-sensitive negative-type silver halide emulsion layer containing yellow coupler. On the other side of support may be provided a non-light-sensitive layer.

To prevent the color fading of a dye image caused by short wavelength active light, an ultraviolet absorbent may be incorporated. For this purpose, thiazolidone, benzotriazole, acrylonitrile, benzophenon compounds and the like are available. Especially, the singly or combinedly used Tinuvin -PS, -20, -326, -327 and -328 (each manufactured by Ciba-Geigy AG) are advantageous.

In embodying the invention, a protective layer, intermediate gelatin layer, and an anti-halation layer on the opposite face of a support may be, in compliance with a specific requirement, formed in addition to the above-mentioned red-, green- and blue-sensitive layers, as well as the non-light-sensitive layer on the opposite face.

In implementing the invention, various photographic additives may be incorporated into the silver halide emulsion being used. The useful optical sensitizers include cyanine, merocyanine, trinuclear or tetranuclear cyanine, styryl, holopolar cyanine, hemicyanine, oxonol and hemioxonol sensitizers, and others.

At the same time, the emulsion may contain often used stabilizing agents such as a compound having an azaindene ring, a heterocylcic compound having a mercapto ring, and others.

The preferred compounds having an azaindene ring include 4-hydroxy-6-methyl-1,3,3a,7-tetraazindene. In relation to heterocyclic compounds to which a mercapto group can be bonded, the example of a ring a heterocyclic compound having a nitrogen atom has are as follows: a pyrazole ring, 1,2,4-triazole ring, 1,2,3-triazole ring, 1,2,3-thiadiazole ring, 1,2,4-thiadiazole ring, 1,2,5-thiadiazole ring, 1,2,3,4-tetraazole ring, pyridazine ring, 1,2,3-triazine ring, 1,2,4-triazine ring, 1,3,5-triazine ring and the like; a ring, formed by condensation of two or three of these rings, such as a triazolotriazole ring, diazaindene ring, triazaindene ring, pentaazindene ring and the like; a phthalazainone ring, indozole ring and others. However, 1-phenyl-5-mercaptotetrazole is especially advantageous.

A wetting agent may be used in compliance with a specific requirement. The examples of such an agent include dihydroxyalkane and the like. Additionally, the examples of an agent useful in improving physical property of the emulsion layers are water-dispersible particle-type high-molecular materials obtainable from the emulsification-polymerization of the following: a copolymer of alkyl acrylate (or, alkyl methacrylate) and acrylic acid (or, methacrylic acid); styrene-maleic acid copolymer; styrene-maleic anhydride-half alkyl ester copolymer; and others. The examples of coating aid include saponin, polyethylene glycol, lauryl ether and the like. Other arbitrarily usable photographic additives include a gelatin plasticizer, surface active agent, ultraviolet absorbent, pH adjusting agent, oxidation inhibitor, anti-static agent, thickner, graininess improver, dye, mordant, whitening agent, development adjuster, matting agent, anti-irradiation dye, and others.

Adequate gelatin (including acid-treated gelatin), or a derivative thereof, may be incorporated into the positive-type silver halide photographic light-sensitive material invention, in accordance with a specific requirement. The examples of preferred gelatin derivative include an acylated gelatin, guanidyl gelatin, carbamyl gelatin, dicyanoethanol gelatin, esterificated gelatin and the like. Such gelatins may be also incorporated into the non-light-sensitive layers. If such layers are formed on the surface of support opposite to where the emulsion layers are formed, such gelatins may be incorporated into such layers.

Additionally, the positive-type silver halide color photographic light-sensitive material of the invention may contain, other than gelatin, other hydrophilic binders in the hydrophilic colloid layers thereof.

The hydrophilic binder may be incorporated, in compliance with a specific requirement, into any of the photographic structural layers such as emulsion layers, intermediate layers, protective layer, filter layer, subbing layer and others. Additionally, the above-mentioned hydrophilic binder may contain an optional arbitrary plasticizer, an antifriction agent and the like. Such gelatins and binders may be, as mentioned previously, incorporated into the non-light sensitive layer. The photographic structural layers of the light-sensitive material of the invention may be hardened with an optional arbitrary hardener. The preferred examples of a useful hardener include chrome salt-, zirconium salt-, halotriazine- vinylsulfon- and acryloyl-hardeners. For the silver bleach type material, aldehyde hardeners such as formaldehyde and mucohalogen acid may be used in addition to the above hardeners.

The positive-type silver halide color photographic light-sensitive material of the invention is prepared by forming various photographic structural layers, in accordance with a requirement, such as the filter layer, intermediate layers, protective layer, subbing layer, anti-halation layer and the like by means of coating. The useful processes of coating include the dip coating process, air doctor coating process, extrusion coating process, slide hopper coating process, curtain flow coating process and others.

When embodying the invention in teh form of a silver dye bleach-type silver halide color photographic light-sensitive material, the applicable methods for color correction masking are disclosed in the specifications of Japanese Patent Publication Open to Public Inspection (hereinafter referred to as Japanese Patent O.P.I. Publication) No. 55944/1971, West German Patents No. 2,831,814, No. 743,535 and No. 898,709, and U.S. Patent No. 2,336,380. If the invention is applied to a method of silver dye bleaching, the useful methods are those disclosed in the specifications of U.S. Patents No. 3,454,402, No. 3,443,953, No. 3,804,630, No. 3,716,368, No. 3,877,949, No. 3,623,874, No. 3,931,142 and No. 4,051,123.

In the case of silver dye bleach type silver halide color photographic light-sensitive material, the cyan-, magenta- and yellow dyes being diffusion-resistant and bleacheable may be contained in the corresponding color-sensitive silver halide emulsion layers, or, otherwise, each color forming dye may be contained in a non-silver halide emulsion layer adjacent to a color-sensitive silver halide emulsion layer corresponding to the dye.

When the invention is applied to a positive-type silver halide color photographic light-sensitive material for the reversal developing process, various processing techniques usually used in treating a reversal-type material can be used for the processing of it. More specifically, the details of a useful color reversal process are as follows: a positive-type silver halide color photographic light-sensitive material comprising a reflective support, provided thereon, a negative-type red-sensitive silver halide emulsion layer to form a cyan dye image, a negative-type green-sensitive silver halide emulsion layer to form a magenta dye image, and a negative-type blue-sensitive silver halide emulsion layer to form a yellow dye iamge, is subjected to the imagewise exposing, whereby a negative silver image is formed by the monochromatic primary developing, then the material is further treated by the processing steps comprising the secondary exposing or fogging treatment, the reversal color developing involving color developing, the bleaching, and the fixing. The light-sensitive material having been treated is stablized by water- rinsing or by stabilizing bath.

The details of treatment when the invention is applied to a silver dye bleach type silver halide color photographic light sensitive material are as follows: the silver halide color photographic light-sensitive material is, after a negative silver image having been formed by the monochromatic primary developing, treated in the bleaching process to bleach dye and silver, and the silver dye bleaching process involving the fixing. For this purpose, the developing may be effected by any technique being capable of silver developing, and, usually, the combined use of hydroquinone as a primary component as well as phenyl-3-pyrazolidone as an auxiliary component is desirable. For bleaching, one useful method is as follows: dye is bleached by using silver as an oxidizing enzyme as well as by combinedly using a strong acid having the pH value less than 2, water soluble additive, oxidizing agent such as m-nitrobenzenesulfonic acid, oxidation inhibitor such as ascorbic acid, and the like. The fixing is carried out to remove silver halide from the layers, and, the fixer used for the bleach-fixing, for example, can be used.

As one application using the positive type silver halide color photographic light-sensitive material of the invention, the color copying with a copying apparatus illustrated in Fig. 3 is available. Fig. 3 shows the copying apparatus to treat a reversal-type silver halide color photographic light-sensitive material, wherein the numeral 1 represents an optical system; the numeral 2 represents a paper feeder; the numeral 3 represents a developing device, and; the numeral 3 represents a dryer device.

The light emitted from an exposure lamp to irradiate an original draft is directed for exposing to the positive-type silver halide color photographic light-sensitive material via a mirror and a lens. The correction of density and hue is effected correspondingly by an aperture and a color filter. By the paper feeder 2, the light-sensitive material housed in the form of roll is cut into a piece having a predetermined size, and exposed in synchronization with the optical system. After the exposing, the piece of light-sensitive material is transferred to the developing device 3. In the developing device 3, the first developing is effected in a first developing bath 31, then the stop-washing is effected in a stop-washing bath 32, whereby the color developing is effected in a color developing bath 33 while the second exposing is exercised with a second exposing light source 33'. Next the light-sensitive material is subjected to the bleach-fixing in a bleach-fixing bath 34, then, to the stabilizing in a stabilizing bath 35. In the example of _{F}ig. 3, the stabilizing bath involves two-bath system comprising 35a and 35b, wherein the counter current method is provided. After the developing, the light-sensitive material is dried in the dryer device, whereby the material subjected to hot air blowing onto the upper and lower surfaces thereof.

The invention is hereinunder described in detail with the reference to the preferred examples. However, the scope and effects of the invention are not limited only to these examples. Naturally, it should be understood that, when there are irregularities whose diameters range from one to 15 mm on the surface of reflective support where silver halide emulsion layers being provided and if the depths of irregularities are less than four vm, such a support is within the scope of the invention, and that, though the diameters of irregularities are less than one mm, and there are artificial irregularities whose depths exceed four µm, such a support is also within the scope of the invention. Furthermore, a support, wherein the surface provided with the emulsion layers is treated so as to satisfy the aforesaid criterion of the invention by providing a subbing layer, is also within the scope of the invention.

### EXAMPLES

The preferred examples embodying the invention are hereinunder described in detail. However, it should be noted that the effects and scope of the invention is not limited only to these examples.

### Example - 1

Firstly, the preparation of the supports, below, is described.

### Preparation of support - 1 (comparison support)

Using the components, above, a hand-made paper having a weighing capacity of 70 g/cm² was prepared and dried with a cylindrical drier at 110 °C. A tub-sizing agent was applied onto the obtained hand-made paper so that the rate of coated carboxy-denatured polyvinyl alcohol was 0.5 g/m². Then the paper was treated with a super calender under a linear pressure of 80 kg/cm. After the surface being treated with the corona discharge, the surface was coated with low density polyethylene (thickness, 25 µm) having a density of 0.93 and containing 15 weight % of anatase-type titanium oxide by means of fusion-extrusion coating at 330 °C, whereby the other surface was treated with the corona discharge, then coated with medium density polyethylene (thickness, 28 µm) having a density of 0.94 by means of the similar coating process at the similar temperature, so as to coat the paper support. This provided a laminated paper having a thickness of 105 µm. Furthermore, the surface of lamination was treated with corona discharge to make the polyethylene hydrophilic.

This support 1, having the thickness of 105 µm, has the irregularities whose depth being 5.8 µm or in excess of 4 µm, which means this support is not in compliance with the criterion of the invention.

### Preparation of support - 2 (support of the invention)

The modification was made on support - 1, whereby the amount of coated carboxy-modified polyvinyl alcohol contained in tab-sizing agent is changed to 2.7 g/m², and the amount of coated cationic starch to 0.6 g/m². After the similar hand-made paper being being treated with a super calender with a linear pressure of 105 kg/cm, whereby polyethylene was laminated in a manner identical to that of support - 1, so as to prepare a laminated paper having a thickness of 102 µm.

This support 2, having a thickness less than 150 µm and the depth of irregularities being 2.8 µm, is a support according to the invention.

### Preparation of support - 3 (support of the invention)

Using polypropyrene synthetic paper Yupo (FPG grade, 110 µm thick) manufactured by Oji Yuka Gosei Co., Otd., a support having a thickness.110 µm and the depth of irregularities being 1.3 µm was prepared. This support - 3 is a support according to the invention.

### Preparation of support - 4 (comparison support)

This support is identical to support - 1, except that its weighing capacity was 160 g/m². The thickness of support, greater than that of support - 1, is 220 µm and the depth of irregularities was 5.8 µm.

The surface irregularities of the above-mentioned supports were measured with a surface roughness tester, Surf Com Model 550 manufactured by Tokyo Seimitsu Co., Ltd. The measuring operation was exercised, using a stylus having a cemented carbide ball with a radii of 0.8 mm, at a scanning speed of 3 mm/sec., and a stylus pressure of 0.5 g. The measurement results for supports - 1, - 2 and - 3 are shown in Fig. 2.

On the surface of each of four types of supports, the emulsion layers below were formed. Then, developing was effected with a uniform exposing light having been color- corrected to grey, then the uneveness of coating was assessed.

The data and assessed results for all the support are listed in Table - 1.

To confirm the effects of the invention, the following emulsions for high-sensitivity reversal color photographic paper were prepared, and applied onto each support of the invention as well as onto each comparison support to form the emulsion layers in the sequence, from bottom upward, of the anti-halation layer, red-sensitive emulsion layer, intermediate layer, green-sensitive emulsion layer, yellow filter layer, blue-sensitive emulsion layer, untraviolet-absorbing layer and protective layer.

### (a) Anti-halation layer

Three % gelatin solution containing five g grey colloidal silver, and three g 2,5-dioctylhydroquinone and surface active agent S - 1 both having been dispersed into dibutylphthalate, was prepared and applied to form a layer, so that the rate of coated colloidal silver was 0.1 g/m².-(b) Red-sensitive emulsion layer

One mol of silver iodo-bromo-chloride emulsion, whose silver halide particles having an average particle diameter of 0.4 µm, comprising three mol % silver iodide and 90 mol % silver bromide was prepared by the neutral conversion process. After washing by a floculating method, five mg sodium thiosulfate and ten mg gold thiocyanate complex were added into the emulsion, then the second ripening was exercised, whereby 100 mg sensitzing dye D - 1 and 50 mg sensitizing dye D - 2 were further added into the emulsion.

Furthermore, into the emulsion were added stabilizing agents T - 1 and T - 2, surface active agent S - 2, and a coupler solution which is a protective-type dispersion containing dibutylphthalate, ethyl acetate, surface active agent S - 2, 2,5-dioctylhydroquinone, and cyan couplers CC - 1 and CC - 2.

The prepared emulsion was applied so that the rate of coated silver was 0.48 g/ₘ².

### (c) First intermediate layer

3.5 % gelatin solution containing five g grey colloidal silver, and three g 2,5-dioctylhydroquinone and surface active agent S - 1 both having been dispersed into dibutylphthalate, was prepared, into which hardener H - 1 being added before coating, and applied to form a layer, so that the rate of coated colloidal silver was 0.1 g/m².

### (d) Green-sensitive emulsion layer

One mol of silver iodo-bromo-chloride emulsion, whose silver halide particles having an average particle diameter of 0.47 µm, comprising three mol % silver iodide and.90 mol % silver bromide was prepared by the neutral conversion process. After washing by the flocculation method, seven mg sodium thiosulfate and 15 mg gold thiocyanate complex were added into the emulsion, then the second ripening was exercised, whereby 90 mg sensitzing dye D - 3 and ten mg sensitizing dye D - 4 were further added into the emulsion. Furthermore, into the emulsion were added one g stabilizing agent T - 1 and 50 mg stabilizing agent T - 2, then, as well as a magenta coupler solution which is a protective-type dispersion containing surface active agent S - 1, 2,5-dioctylhydroquinone, magenta coupler MC - 1, dioctylphthalate and ethyl acetate. Gelatin, and hardener H - 1 were also added into the emulsion, which was applied so that the rate of coated silver was 0.4 g/ₘ².

### (e) Yellow filter layer

Yellow colloidal silver was added into a solution which is a protective-type dispersion containing surface active agent S - 1 and 2,5-dioctylhydroquinone, thereinto surface active agent S - 2 and hardener _{H} - 1 were further added, then the prepared emulsion was applied so that the rate of coated colloidal silver was 0.12 g/m².

### (f) Blue-sensitive emulsion layer

One mol of silver iodo-bromide emulsion, whose silver halide particles having an average particle diameter of 0.7 µm, containing 3.6 mol % silver iodide was prepared by the neutral conversion process. After washing by the locculation method 20 mg sodium thiosulfate and 15 mg gold thiocyanate complex were added into the emulsion, then the second ripening was exercised, whereby 18 mg sensitzing dye D - 5 was further added into the emulsion. Furthermore, into the emulsion were added stabilizing agents T - 1 and T - 3, then, as well as a solution which is a protective-type dispersion containing surface active agent S - 1, 2,5-dioctylhydroquinone, yellow coupler YC - 1, ethyl acetate and dioctylphthalate. Gelatin and hardener H - 1 were also added into the emulsion, which was applied so that the rate of coated silver was 0.58 g/ₘ²_{.}

### (g) Ultraviolet absorbing layer

Gelatin solution, which is a protective-type dispersion containing surface active agent S - 1, Tinuvin 328, Tinuvin 320 (ultraviolet absorbents manufactured by Ciba-Geigy _{AG}), dibutylphthalate and ethyl acetate, was prepared and applied so that the rate of coated Tinuvin was 0.5 g/m².

### (h) Protective layer

Gelatin solution containing colloidal silica, coating auxiliary S - 3 and hardener H - 2 was applied so that the rate of coated gelatin was 0.8 g/m².

The materials used, above, are listed below.

Each light-sensitive material having been provided with coating and dried was subjected to heat-aging at 40 °C for five days, whereby subjected to uniform exposing, then the reverse developing was exercised in the following manner, so as to assess the uneven density of image.

### Processing steps

The composition of each processing solution is as follows. <First developer composition>

Water was added to the above ingredients to prepare one ℓ solution.

### <Color developer composition>

Water was added to the above ingredients to prepare one ℓ solution.

### <Bleach-fixer composition>

Water was added to the above ingredients to prepare one ℓ solution.

As indicated by Table 1, the results of assessement, on the uneven density of image, obtained by using sample light-sensitive materials, show that the light-sensitive materials of the invention are free from the uneveness in density of image, and, therefore, can provide the uniform quality of image, as well as an excellent image. In contrast, the light-sensitive material using comparison support - 1, which is not in compliance with the invention, shows greater uneveness of density, and, therefore, its image quality was unsatisfactory.

In the table, above, the symbols for assessment of uneven density are as follows:
xx Great uneveness, and, unsatisfactory
o Satisfactory
o Excellent

As shown in Table - 1, supports - 1 and - 2 respectively have flocs of pulp caused while the pulp is formed into sheet, and the irregularity sizes (maximum diameters of the irregularities) range from four through six mm. The degree of uneveness in density depends on the depth of irregularity. Accordingly, support - 2 (the irregularity depth of which being 2.8 µm) of the invention showed no uneven density, and attained favorable results. Furthermore, having the irregularity with a depth of 1.3 µm, support - 3 of the invention showed by far the better results. At the same time, with support - 4, though the irregularity depth being 5.8 µm and rather large, the uneveness in density did not occur, because the thickness of support, rather large, was 220 µm. However, being thick, support - 4 posed disadvantages for filing, because of its bulkiness.

### Example - 2

With this example, the following emulsions for color photographic paper were prepared, and the layers were formed, by coating, respectively on the supports of the invention and the comparison support, in the sequence of, from the bottom upeards, the red-sensitive emulsion layer, first intermediate layer, green-sensitive emulsion layer, yellow filter layer, blue-sensitive emulsion layer and protective layer.

### (a) Red-sensitive emulsion layer

One mol of silver iodo-bromo-chloride emulsion, whose silver halide particles having an average particle diameter of 0.4 µm, comprising 0.7 mol % silver iodide and 70 mol % silver bromide was prepared by the neutral conversion process. After washing by the flocculation method, sodium thiosulfate and gold thiocyanate complex were added into the emulsion, then the second ripening was exercised, whereby sensitzing dyes D - I and D - 2 were further added into the emulsion. Furthermore, into the emulsion were added stabilizing agents T - 1 and T - 2, surface active agent S - 2 and a cyan dye CD - 1, then, gelatin was added into the emulsion, which was applied so that the rate of coated silver was 0.5 g/m² and the similar rate of cyan dye was 0.10 g/m².

### (b) First intermediate layer

Gelatin solution containing surface active agent S - 2 and hardener H - 1 was prepared and applied to form a layer, so that the rate of coated gelatin was 1.5 g/m².

### (c) Green-sensitive emulsion layer

One mol of silver iodo-bromo-chloride emulsion, whose silver halide particles having an average particle diameter of 0.51 pm, comprising 0.6 mol % silver iodide and 90 mol % silver bromide was prepared by the neutral process. After washing by the flocculation method, sodium thiosulfate and gold thiocyanate complex were added into the emulsion, then the second ripening was exercised, whereby sensitzing dye _{D} -3 was further added into the emulsion. Furthermore, into the emulsion were added stabilizing agents T - 1 and T - 2, then, as well as surface active agent S - 2 and magenta dye _{MD} - 1, whereby gelatin was added into the emulsion, which was applied so that the rate of coated silver was 0.55 g/m² and the similar rate of coated magenta dye MD - 1 was 0.11 g/m².

### (d) Yellow filter layer

Gelatin solution containing surface active agent S - 2, hardener H - 2 and colloidal silver was prepared and applied so that the rate of coated colloidal silver was 0.13 g/m².

### (e) Blue-sensitive emulsion layer

One mol of silver iodo-bromide emulsion, whose silver halide particles having an average particle diameter of 0.7 pm, containing 1.6 mol % silver iodide was prepared by the conversion process. After washing by the flocculation method, sodium thiosulfate and gold thiocyanate complex were added into the emulsion, then the second ripening was exercised, whereby sensitzing dye D - 5 was further added into the emulsion. Furthermore, into the emulsion were added stabilizing agents T - 1 and T - 3, surface active agent S - 2, yellow dye _{Y}D - 1, hardener H - 1 and gelatin. The emulsion was applied so that the rate of coated silver was 0.7 g/ₘ².

### (f) Protective layer

Gelatin solution containing surface active agent _{S} - 2 and hardener H - 2 was prepared and applied so that the rate of coated gelatin was 1.5 g/ₘ².

The materials used, above, are listed below. Processing steps were as follows.

The composition of each processing solution is as follows. <Developer>

Water amount to prepare one ℓ solution <Bleaching solution>

Water amount to prepare one t solution <Fixing solution>

Water amount to prepare one k solution

As a result, similarly to Example - 1, being free from the density uneveness of image, the light=sensitive materials of the invention satisfactorily provided a high-quality image. Example - 3

The following emulsions for color photographic paper were prepared, and the layers were formed, by coating, respectively on the supports of the invention and the comparison support, in the sequence of, from the bottom upwards, the gelatin subbing layer, cyan dye layer, red-sensitive emulsion layer, magenta dye layer, green-sensitive emulsion layer, yellow dye layer, blue-sensitive emulsion layer and protective layer.

### (a) Gelatin subbing layer

Gelatin solution containing surface active agent S - 2 was applied, so that the rate of coated gelatin was 2.0 g/m²,

### (b) Cyan dye layer

Gelatin solution containing surface active agent S - 2, hardener H - 1 and cyan dye CD - 1 was applied so that the rate of coated cyan dye C_{D} - 1 was 0.₁4 g/m².

### (c) Red-sensitive emulsion layer

One mol of silver iodo-bromo-chloride emulsion, whose silver halide particles having an average particle diameter of 0.4 µm, comprising 0.7 mol % silver iodide and 70 mol % silver bromide was prepared by the neutral conversion process. After washing by the flocculation method, sodium thiosulfate and gold thiocyanate complex were added into the emulsion, then the second ripening was exercised, whereby sensitzing dyes D - 1 and D - 2 were further added into the emulsion. Furthermore, into the emulsion were added stabilizing agents T - 1 and T - 2, surface active agent S - 2 and a cyan dye CD - 1, and, thereinto gelatin was added, and the emulsion was applied so that the rate of coated silver was 0.5 g/m².

### (d) Magenta dye layer

Gelatin solution containing surface active agent S - 2, hardener H - 1 and magenta dye MD - 1 was prepared and applied to from a layer, so that the rate of coated magenta dye MD - 1 was 0.18 g/ₘ²_{.}

### (e) Green-sensitive emulsion layer

One mol of silver iodo-bromo-chloride emulsion, whose silver halide particles having an average particle diameter of 0.51 pm, comprising 0.6 mol % silver iodide and 90 mol % silver bromide was prepared by the neutral process. After washing by the flocculation method, sodium thiosulfate and gold thiocyanate complex were added into the emulsion, then the second ripening was exercised, whereby sensitzing dye D - 3 was further added into the emulsion. Furthermore, into the emulsion were added stabilizing agents T - 1 and T - 2, then, as well as surface active agent S - 2 and magenta dye MD - 1, whereby gelatin was added into the emulsion, which was applied so that the rate of coated silver was 0.55 g/m².

### (f) Yellow dye layer

Gelatin solution containing surface active agent S - 2, hardener H - 2 and yellow dye was prepared and applied so that the rate of coated yellow dye was 0.10 g/m².

### (g) Blue-sensitive emulsion layer

One mol of silver iodo-bromide emulsion, whose silver halide particles having an average particle diameter of 0.7 µm, containing 1.6 mol % silver iodide was prepared by the conversion process. After washing by the flocculation method, sodium thiosulfate and gold thiocyanate complex were added into the emulsion, then the second ripening was exercised, whereby sensitzing dye D - 5 was further added into the emulsion. Furthermore, into the emulsion were added stabilizing agents T - 1 and T - 3, surface active agent S - 2, hardener H - 1 and gelatin. The emulsion was applied so that the rate of coated silver was 0.7 g/ₘ².

### (h) Protective layer

Gelatin solution containing surface active agents S - 2 and hardener H - 2 was prepared and applied so that the rate of coated gelatin was 1.5 g/m².

The developing was exercised in a manner identical to that of Example - 2.

The assessment results are listed in Table - 2.

Similarly to Example - 2, the samples respectively comprising the support of the invention, whose support being thin, were free from the uneveness in density and accordingly attained satisfactory results.

In this table, the symbols representing the assessment results have meanings identical to those of Example - 1.

### Example - 4

The following layers were sequentially formed, by coating, respectively on the supports of the invention and the comparison support.

### First layer

Blue-sensitive silver halide emulsion containing yellow coupler (chloro-bromide silver emulsion involving 90 mol % silver bromide, and containing gelatin at a rate of 300 g per mol silver halide, as well as yellow coupler YC - 1 having been dissolved and dispersed into dibutylphthalate at a rate of 0.5 mol per mol silver halide) was applied and dried so that the rate of coated gelatin was 2 g/m².

### Second layer

A first intermediate layer (gelatin layer; the rate of coated gelatin being 1.5 g/m2).

### Third layer

Green-sensitive silver halide emulsion containing magenta coupler (chloro-bromide silver emulsion involving 80 mol % silver bromide, and containing gelatin at a rate of 400 g per mol silver halide, as well as magenta coupler MC - I having been dissolved and dispersed into dibutylphthalate at a rate of 0.3 mol per mol silver halide) was applied and dried so that the rate of coated gelatin was 2 g/ₘ².

### Fourth layer .

A second intermediate layer containing ultraviolet absorbent: example ultraviolet absorbent UV - 1 having been dissolved into 20 g dibutylphthalate was dispersed into gelatin, which was applied and dried, so that the rate of coated ultraviolet absorbent was 0.6 g/m² and the rate of coated gelatin was 1.5 g/ₘ².

### Fifth layer

Red-sensitive silver halide emulsion containing cyan coupler (chloro-bromide silver emulsion involving 80 mol % silver bromide, and containing gelatin at a rate of 300 g per mol silver halide, as well as cyan coupler CC - 2 having been dissolved and dispersed into dibutylphthalate at a rate of 0.4 mol per mol silver halide) was applied and dried so that the rate of coated gelatin was 20 g/m².

### Sixth layer

A protective layer containing ultraviolet absorbent: example ultraviolet absorbent UV - 1 having been dissolved into dibutylphthalate was dispersed into gelatin, which was applied and dried, so that the rate of coated ultraviolet absorbent was 0.4 g/m² and the rate of coated gelatin was 1.5 g_{/m}²_{.}

After uniform-exposing, each sample was subjected to the color developing in compliance with the following steps.

The conditions of developing were as follows.

### Color developer composition

N-ethyl-N-β-methanesulfonamideethyl-3-methyl-e-aminoaniline

Water was added to the above ingredients to prepare one ℓ solution, which was treated with sodium hydroxide to adjust the pH value to 10.0.

### Bleach-fixer composition

Water was added to the above ingredients to prepare one ℓ solution, which was treated with sulfuric acid to adjust the pH value to 10.0.

### Oxidation-reduction potential: - 70 mv

The test results are listed in Table - 3.

In the table, above, the symbol representing the result of assessment for density uneveness is as follows:
o Satisfactory

As can be understood from the results in Table - 3, the uneveness of density found on support - 1 in Example - 1 was not found in this example. This means that the density uneveness is readily visible when the same support is used in a reversal positive-type silver halide photographic light-sensitive material, and, in contrast, that the nature of support exerts smaller influence on the visibility of uneveness if the same support is used in a negative-type silver halide photographic light-sensitive material.

### Example - 5

Respectively using the samples 1, 2 and 3 prepared in Example - 1, a specific original color draft was duplicated with a copying apparatus illustrated in Fig. 3. A duplicated image obtained with sample 1 showed the occurrence of serious density uneveness. In contrast, the density uneveness on sample 2 was small and allowable for practical use. Furthermore, sample 3 was almost free from the density uneveness.

Conditions of the reversal developing effected in the copying apparatus were identical to those in Example - 1.

Though having a thin support, the positive-type silver halide color photographic light-sensitive material of the invention is capable of forming a high-quality color image free from density uneveness, and, therefore, is suitable for providing a thin duplicate.

## Claims

1. A positive-type silver halide color photographic light-sensitive material, comprising a reflective support, provided thereon, a negative-type red-sensitive silver halide emulsion layer to form a cyan dye image, a negative-type green-sensitive silver halide emulsion layer to form a magenta dye image and a negative-type blue-sensitive silver halide emulsion layer to form a yellow dye image, and the dye image density is formed as a negative function in proportion to the amount of image exposure, wherein said reflective support has a thickness of 80to 150 µm, and when there are irregularities having diameters ranging from one to 15 mm on the surface thereof where said silver halide emulsion layers are disposed, the depths of said irregularities are less than 4 pm.

2. A positive-type silver halide color photographic light-sensitive material of Claim 1, wherein said photographic material is a reversal-type said silver halide color photographic light-sensitive material.

3. A positive-type silver halide color photographic light-sensitive material as claimed in Claim 1, wherein said photographic material is a silver dye bleach type silver halide color photographic light-sensitive material.
